

## UNITED STATES PATENT OFFICE.

EDMUND PAKULLA, OF REMSCHEID, GERMANY, ASSIGNOR, BY MESNE ASSIGNMENTS, TO DEUTSCHE EDELSTAHLWERKE AKTIENGESELLSCHAFT, OF BOCHUM, GERMANY, A CORPORATION OF GERMANY.

## STEEL ALLOY AND PROCESS OF MAKING THE SAME.

No Drawing. Application filed September 18, 1924, Serial No. 738,525, and in Germany June 9, 1923.

My invention relates to steel alloys and the process of making the same, and more particularly to alloys of the character and composition of high speed steels. As is known to those skilled in the art high speed steels such as are now in use have very poor magnetic properties. The object of the improvements is to manufacture a steel of the character and composition of high speed steels which shows valuable magnetic properties adapting the same to the manufacture of permanent magnets, and with this object in view I heat ordinary high speed steel at a temperature a little higher than "lowering temperature", and I quench the same in oil, petroleum, or other suitable quenching media. According to Swinden, in the Journal of the Iron and Steel Institute, 1907, volume 1, page 319, "lowering temperature" is understood to be the temperature at which certain sorts of steel must be heated in order to lower the  $Ar_1$ -transformation when cooling the steel.

Particularly the values of the coercive force imparted to the high speed steel by my improved process are such that my improved steel is superior in quality to good chromium or tungsten steel.

Further, I have found that the magnetic properties of high speed steel are improved by adding cobalt to the steel, the coercive force of the steel being increased in a degree as the proportion of cobalt in the steel is increased.

Example 1.—A high speed steel containing 0.7% C, 12% Wo and 4% Cr has been heated at  $1100^\circ$  centigrade and quenched in oil. It showed the following magnetic values: remanence 6550, coercive force 91.5,

product of remanence and coercive force  $599 \times 10^3$ .

Example 2.—A high speed steel containing 0.7% C, 0.3% Mn, 0.25% Si, 7% Mo, 4.5% Cr, 1.5-2% Co was heated at  $1150^\circ$  centigrade and quenched in oil. It showed a remanence of 7000, a coercive force of 90, and the product of both  $630 \cdot 10^3$ .

Example 3.—A high speed steel containing 0.8% C, 7% Mo, 4% Cr, and 5% Co, after being heated and quenched, showed a remanence of 6800 to 7500, a coercive force of 100 to 110, and the average product of both was  $730 \cdot 10^3$ .

Example 4.—A high speed steel containing 0.6 to 0.8% C, 0.5% Mn, 0.25% Si, 4 to 5% Cr, 7 to 8% Mo, 1 to 2% Co, 0.5% V was heated at  $1150^\circ$  centigrade, and quenched in oil. It showed the following magnetic values: remanence 7000, coercive force 90.

## I claim:

1. The process of manufacturing permanent magnets, which consists in heating high speed steel containing chromium and at least one of the elements tungsten, molybdenum or cobalt at a temperature above lowering temperature, and quenching the same in mild non-aqueous hardening agents.

2. The process of manufacturing permanent magnets, which consists in heating high speed steel containing 0.6 to 0.8% C, 0.5% Mn, 0.25% Si, 4 to 5% Cr, 7 to 8% Mo, 1 to 2% Co and 0.5% V at a temperature of  $1150^\circ$  centigrade, and quenching the same as set forth above.

In testimony whereof I hereunto affix my signature.

EDMUND PAKULLA.